

July 5, 1955

H. E. GRESHAM ET AL  
NICKEL CHROMIUM ALLOYS HAVING HIGH CREEP  
STRENGTH AT HIGH TEMPERATURES  
Filed May 23, 1949

2,712,498



BY

INVENTORS.  
HAROLD E. GRESHAM  
ADAM DUNLOP  
MARCUS A. WHEELER  
Kenyon & Kenyon  
ATTORNEYS.

1

2,712,498

## NICKEL CHROMIUM ALLOYS HAVING HIGH CREEP STRENGTH AT HIGH TEMPERATURES

Harold Ernest Gresham, Little Eaton, Adam Dunlop, Alvaston, and Marcus Alan Wheeler, Darley Abbey, England, assignors to Rolls-Royce Limited, Derby, England, a British company

Application May 23, 1949, Serial No. 94,816

Claims priority, application Great Britain June 1, 1948

8 Claims. (Cl. 75—171)

Our invention relates to alloys from which to make engineering parts capable of withstanding great stress at high temperatures, ranging for instance between 700° and 1050° C. As examples of such engineering parts we may mention the blades and other parts of internal combustion gas turbines. Claim is hereby made for the benefit of the filing date of patent application numbered 14,823 of 1948 filed in Great Britain June 1, 1948.

In our research work on alloys of this type we started from the nickel-chromium base alloys which are commonly used in the productions of high duty engine parts and which often contain cobalt and as hardening constituents aluminum and titanium. Like other workers in this field, we have had the experience that sometimes quite trifling differences in the constitution of this type of alloys—differences such as will normally spring up even in careful foundry practice—lead to alloys of widely divergent properties so that it appeared to be impossible to predicate with certainty the quality of an engineering part made out of an alloy of this type, until it had been actually tested.

The drawing annexed to and forming part hereof is a chart on which Time to Fracture is plotted against "Balance Factor" (hereinafter defined) for a series of twelve alloys all containing the same constituent metals but in differing proportions and having different "balance factors."

During our studies in this special field we made a surprising discovery which, we believe, is adapted to lift the production of high duty engineering parts of the kind here in view from a stage of comparative uncertainty to the level of an altogether controllable production leading to predetermined properties of the products.

We have found that there exists a definite correlation between the properties of a nickel-chromium-cobalt alloy, in which the cobalt is contained within the range of about 10 and 40 per cent by weight of the complete alloy, and chromium within the range of 10 and 30 per cent and which contains, besides aluminum and titanium, also molybdenum within the ranges of 2 to 18 per cent molybdenum, 0.2 to 8.6 per cent aluminum and 0.2 to 4.4 per cent titanium—and the total percentage of molybdenum, aluminum and titanium present.

We have found that this type of alloys with fully predictable properties will be produced, if the percentages of the three alloying metals Mo—Al—Ti are so chosen that by adding once the percentage of molybdenum plus twice the percentage of aluminum plus four times the percentage of titanium, a figure is reached which ranges between 16 and 20.

The range of 16–20 arrived at according to the formula

$$1 \times \text{percent Mo} + 2 \times \text{Al} + 4 \times \text{percent Ti}$$

we will call for convenience "the balance factor."

One of the principal advantages gained by the use of a composition balanced in accordance with our discovery is the safe control of the creep strength. For it is known that a number of well known alloys, in current use where high creep strength is required, suffer from considerable variation in their properties, a circumstance which we found to be due to the use of unbalanced compositions.

The great advantages resulting in the use of our "bal-

2

ance factor" formula are illustrated by the addition of molybdenum, aluminum and titanium in the following examples, in each of which the alloy contains 20% chromium and 20% cobalt, the balance being nickel. These alloys were tested at 815° C. under a load of 15 long tons/sq. in.

|                        | (a)  | (b)   | (c)   | (d)   | (e)   | (f)   | (g)   | (h)   |
|------------------------|------|-------|-------|-------|-------|-------|-------|-------|
| 10 Molybdenum, percent | 15.5 | 5.94  | 6.10  | 6.12  | 3.50  | 5.92  | 6.00  | 0.84  |
| Aluminum, percent      | 0.9  | 3.75  | 0.96  | 0.49  | 1.22  | 0.87  | 0.85  | 0.48  |
| Titanium, percent      | 0.2  | 0.9   | 2.76  | 2.58  | 2.55  | 1.80  | 2.04  | 2.46  |
| Balance Factor         | 18.1 | 17.04 | 19.06 | 17.42 | 16.26 | 14.86 | 15.86 | 12.64 |
| Hours to Fracture      | 80   | 170   | 143   | 117   | 135   | 17    | 34    | 38    |

It will be noted that, when the balance factor is below 16, as is the case in examples f, g, and h, the period of time which elapsed before fracture, is short. On the other hand examples a, b, c, d and e, clearly indicate the great advantage gained by the use of our formula in connection with alloys of widely different compositions.

The use of our formula is equally of great value in controlling the properties of alloys held to a much narrower range of composition. In making a considerable number of casts from alloys of the type containing, besides 20% Cr and 20% Co, 6 per cent Mo, 0.9 per cent Al and 2.4 per cent Ti, the balance being Ni, in varying the percentage of Mo by  $\pm 0.4$  per cent, of Al by  $\pm 0.3$  per cent and of Ti  $\pm 0.3$  per cent, we found that, if all errors were towards the minus side and the balance factor dropped to 15.2, the creep strength was poor. On the other hand, whenever one of the three elements kept on the higher level, the creep properties were greatly improved.

A series of twelve nickel alloys were prepared having the approximate composition 20% chromium and 20% cobalt, while the percentage of Mo ranged from 5.5 to 6.5, that of Al from 0.4 to 1.2, that of Ti from 2.2 to 2.7. Such ranges of composition would be expected to yield alloys having very much the same properties. However the very sensitive creep test brought to light great differences in the behaviour of different alloys and as plotted in the form of twelve points marked "x" on the chart hereto annexed, the life to fracture (hours) of said alloys under the abovementioned test conditions (15 long tons/sq. in. at 815° C.) ranged from a low of about 14 to a high of about 190. Such variations in the creep results are well known to metallurgists. They constitute a great problem in the bulk production of creep-resisting alloys. However, as soon as these small variations of composition are examined in reference to our formula, their real significance becomes obvious and the need for a balanced composition becomes apparent. On the accompanying chart the above-mentioned twelve alloys have been plotted according to their respective "balance factors," which varied from about 15 to about 19.6. When thus plotted it is at once seen that a relationship exists between a balance factor ranging from 16 to 20 and the attainment of high creep strength. The line 10 which is drawn on the chart following generally the rising trend of the several points marked "x" does not represent the results of any tests other than those indicated by the points themselves; it is intended only to emphasize and point out the above-mentioned relationship which we have discovered. By using the formula, one is in the position to choose a composition which, while allowing for normal variation during manufacture, results in consistently high creep properties being obtained.

If the "balance factor" exceeds 20, hot working of the alloys becomes difficult. Therefore the use of our formula again ensures that an alloy will be adapted to be satisfactorily hot-worked.

As to the presence of other metals, the nickel may be replaced up to 10 per cent by vanadium, and there may further be present:

|           | Per cent |
|-----------|----------|
| Niobium   | 0-4      |
| Manganese | 0-2      |
| Silicon   | 0-1      |
| Iron      | 0-5      |
| Carbon    | 0-0.5    |
| Nitrogen  | 0-0.25   |

While niobium may be beneficial, since it improves creep strength, and manganese and silicon are added mainly as cleansing elements, iron, which occurs as an impurity in many commercial metals, should be kept as low as possible. Carbon, also present as an impurity, should also remain within the limits indicated above.

For cleansing and de-oxidation purposes up to 0.5, in all, of the elements calcium, magnesium, cerium and other rare earth metals or misch-metal may be present.

The alloys should be heat-treated to increase hardness and strength and assist in fabrication. A suitable heat-treatment includes preliminary heating at 1050 to 1250° C. during 2 to 20 hours, and this should be followed by reheating at 700-1000° C. for 2 to 50 hours to produce the highest degree of hardening.

The wide control of hardness by a combination of balanced composition and heat treatment is an important feature of our invention.

For maximum creep strength it is essential to compound the alloy according to the formulas given above so as to ensure that the "balance factor" remains within the range of 16-20 and that the molybdenum, aluminum and titanium are all present simultaneously.

We wish to point out that various changes may be made in certain substances, steps and figures hereabove mentioned without departing from our invention or sacrificing the advantages thereof.

We claim:

1. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, each of the three hardening elements molybdenum, aluminum and titanium within the respective approximate ranges 2% to 18% molybdenum, 0.2% to 8.6% aluminum and 0.2% to 4.4% titanium, the impurities iron and carbon not exceeding about 5% iron and 0.5% carbon, and the balance essentially nickel, said alloy being characterized in that the sum of the percentage of molybdenum plus twice the percentage of aluminum plus four times the percentage of titanium equals a figure within the range of 16 to 20.

2. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, each of the three hardening elements molybdenum, aluminum and titanium within the respective approximate ranges 2% to 18% molybdenum, 0.2% to 8.6% aluminum and 0.2% to 4.4% titanium, the impurities iron and carbon not exceeding about 5% iron and 0.5% carbon, up to 10% vanadium, and the balance essentially nickel, said alloy being characterized in that the sum of the percentage of molybdenum plus twice the percentage of aluminum plus four times the percentage of titanium equals a figure within the range of 16 to 20.

3. A hot-workable nickel-chromium base alloy having a life to fracture under load of 15 long tons per square inch at 815° C. substantially in excess of 38 hours, said alloy consisting by weight approximately of 20% cobalt, 20% chromium, each of the three hardening elements molybdenum, aluminum and titanium within the respective approximate ranges 5.5% to 6.5% molybdenum, 0.4% to 1.2% aluminum and 2.2% to 2.7% titanium,

the impurities iron and carbon not exceeding about 5% iron and 0.5% carbon, and the balance essentially nickel, said alloy being characterized in that the sum of the percentage of molybdenum plus twice the percentage of aluminum plus four times the percentage of titanium equals a figure within the range of 16 to 20.

4. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, 15.5% molybdenum, 0.9% aluminum, 0.2% titanium, and the balance essentially nickel, said alloy being characterized in that the sum of the percentage of molybdenum plus twice the percentage of aluminum plus four times the percentage of titanium equals a figure within the range of 16 to 20.

5. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, 5.94% molybdenum, 3.75% aluminum, 0.9% titanium, and the balance essentially nickel, said alloy being characterized in that the sum of the percentage of molybdenum plus twice the percentage of aluminum plus four times the percentage of titanium equals a figure within the range of 16 to 20.

6. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, 6.10% molybdenum, 0.96% aluminum, 2.76% titanium, and the balance essentially nickel, said alloy being characterized in that the sum of the percentage of molybdenum plus twice the percentage of aluminum plus four times the percentage of titanium equals a figure within the range of 16 to 20.

7. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, 6.12% molybdenum, 0.49% aluminum, 2.58% titanium, and the balance essentially nickel, said alloy being characterized in that the sum of the percentage of molybdenum plus twice the percentage of aluminum plus four times the percentage of titanium equals a figure within the range of 16 to 20.

8. A hot-workable nickel-chromium base alloy having a life to fracture under load of 15 long tons per square inch at 815° C. substantially in excess of 38 hours, said alloy consisting by weight approximately of 10% to 40% cobalt, 10% to 30% chromium, 3.50% molybdenum, 1.22% aluminum, 2.58% titanium, and the balance essentially nickel, said alloy being characterized in that the sum of the percentage of molybdenum plus twice the percentage of aluminum plus four times the percentage of titanium equals a figure within the range of 16 to 20.

#### References Cited in the file of this patent

##### UNITED STATES PATENTS

|           |                      |               |
|-----------|----------------------|---------------|
| 2,048,165 | Pilling et al. ----- | July 21, 1936 |
| 2,103,500 | Touceda -----        | Dec. 28, 1937 |
| 2,246,078 | Rohn et al. -----    | June 17, 1944 |
| 2,398,678 | Thielemann -----     | Apr. 16, 1946 |
| 2,403,128 | Scott et al. -----   | July 2, 1946  |
| 2,423,738 | Thielemann -----     | July 8, 1947  |
| 2,570,194 | Bieber et al. -----  | Oct. 9, 1951  |

##### FOREIGN PATENTS

|    |         |                     |               |
|----|---------|---------------------|---------------|
| 70 | 583,845 | Great Britain ----- | Jan. 1, 1947  |
|    | 607,616 | Great Britain ----- | Sept. 2, 1948 |

##### OTHER REFERENCES

Knight, Treatise in Materials and Methods, June 1946, pages 1557-1563; 1562 relied upon.